

1

3,165,424

TREATMENT OF CELLULOSE TEXTILES  
Josef König, Siegburg, Rhineland, and Egon N. Petersen,  
Neumünster, Germany, assignors to Phrix-Werke  
Aktiengesellschaft, Hamburg, Germany  
No Drawing. Filed Apr. 6, 1960, Ser. No. 20,268  
Claims priority, application Germany, Apr. 6, 1959,

P 22,536

11 Claims. (Cl. 117—139.4)

The present invention relates to the treatment of textile materials so as to render the same crease resistant and wrinkle resistant, and more particularly to the treatment of cellulose materials to impart crease resistant and wrinkle resistant properties to the same while maintaining the strength of the material.

It is known to treat textile materials, such as threads, fibers, yarns and webs made of material or regenerated cellulose, with acidic mixtures of water-soluble substances which can be transformed under action of heat into an insoluble resin-like state, in order to render the textile materials crease-proof or to stabilize the textile materials against shrinkage during washing. It is known to impregnate textile materials of the above described type with solutions of aldehydes such as formaldehyde or glyoxal which contain acidic catalysts, or pre-condensates of urea-formaldehyde or melamine-formaldehyde, these solutions being condensed on the material to become insoluble under the action of heat. Such products tend to render the textile material stiff and brittle and/or to impair the strength characteristics of the textile material.

According to a different finishing method, the textile material is coated with cellulose ethers of different kinds. If such ethers possess a low degree of alkylation so that they are soluble only in alkalies but not in water, they are undesirable in the treatment of textile materials made of cellulose because they require a comparatively high concentration of an alkali. The alkali causes swelling of the material and thereby prevents rapid penetration of the cellulose ether. Cellulose ethers with a higher degree of alkylation possess the advantage that they are soluble in water. However, when using such cellulose ethers, the problem arises that they must be made water-insoluble in order to insure that the textile materials treated with such ethers remain washproof.

It is also known to utilize solely alkali-soluble, i.e., water-insoluble cellulose ethers, such as simple alkyl ethers, carboxyl ethers, mixed alkyl-oxyalkyl ethers or mixed alkyl-carboxyalkyl ethers together with solutions which, upon heating, produce synthetic resins. Such prior methods were found impractical in actual use partly because the individual components of such mixtures are often incompatible so that one obtain turbid, easily flocculable suspensions. Simple as well as mixed etherified alkyl cellulose products, such as methyl cellulose or methyl ethyl cellulose, which preferably should be completely etherified because otherwise they are not sufficiently water-soluble, are not suitable because they cannot prevent the stiffness and brittleness of a textile material caused by the deposition of synthetic resins. Also, such alkyl cellulose substances reduce the crumbling strength (creasing resistance) of the synthetic resin impregnation. Oxalkyl and carboxyalkyl celluloses, on the other hand, have the disadvantage that they cannot be fixed in a washproof manner.

It is accordingly a primary object of the present invention to provide a process of treating cellulose materials so as to achieve improved crease resistance and wrinkle resistance.

It is another object of the present invention to provide a method of treating cellulose materials with a treating

2

liquor so that the treated cellulose material has good crease resistance and wrinkle resistance along with high strength characteristics and a good feel.

In general the present invention provides a method of providing crease resistance to cellulose material by a procedure which avoids all of the above and other enumerated disadvantages of the prior art.

Other objects and advantages of the present invention will be apparent, from a further reading of the specification and of the appended claims.

With the above and other objects in view, the present invention mainly concerns a method of improving the crease resistance and non-shrinking properties of cellulose textiles, comprising the steps of treating a cellulose textile material with an acid aqueous liquor containing in solution a water soluble resin-forming substance which upon heating to a predetermined temperature below the temperature at which damage to the cellulose textile material occurs is transformed into an insoluble resinous substance, the water soluble resin-forming substance containing hydroxyl groups, and also containing in solution a water soluble alkyloxy cellulose containing free hydroxyl groups, and heating the thus treated cellulose textile material to the predetermined temperature so as to convert the water soluble resin-forming substance into an insoluble resinous substance and to cause cross linking reaction between the same and the water soluble alkyloxy cellulose, thereby forming a treated cellulose textile material having improved properties.

The treating of the textile material may be carried out by spraying the same with the aqueous liquor, but is preferably accomplished by immersing the textile material in the liquor. The heating temperature is generally above 100° C. and is most preferably at a temperature between 100 and 150° C.

The method of the present invention makes it possible to improve textile material of the cellulose type with respect to the crease resistance thereof while retaining the properties of strength and also while giving to the textile material a good feel. The method of the present invention is particularly advantageous in that the crease resistance which is imparted to the textiles remains even after laundering. This is achieved in accordance with the present invention by the use of the cellulose mixed ether, that is the alkoxy cellulose which contains free hydroxyl groups in the cellulose molecule, these free hydroxyl groups reacting with and cross linking the resin-forming substance, for example the dimethylol urea. The cellulose mixed ether also has the advantage of a good water solubility and the possibility of producing stable, non-flocculating solutions.

The alkyloxy alkyl celluloses which are utilized in the present invention are produced by reacting an alkali cellulose with about 1 mol of a common alkylating agent and about 3 mols of a common alkoxyalylating agent, calculated per each mol of glucose anhydride of the cellulose. For example a suitable mixed ether for the treatment solution is ethoxyethyl cellulose produced by etherifying alkali cellulose with about 1 mol of ethyl halogenide and about 3 mols of ethylene oxide calculated per each mol of glucose anhydride whereby the resulting alkyloxy alkyl cellulose contains ether groups and free hydroxyl groups. Particularly good properties of the treated textile with respect to crease or wrinkle resistance and good feel are achieved by maintaining the mol ratios of the produced cellulose ether as set forth above.

Celluloses of this type are suitable as starting material for the production of the mixed cellulose ethers of the present invention. As alkylating agent it is possible to use a lower alkyl halogenide such as methyl bromide, methyl chloride, ethyl bromide and ethyl chloride. As alkoxyalylating agent it is possible to use a lower alkylene

oxide such as ethylene oxide, propylene oxide, ethylene chlorohydrin and the like.

The treatment solution should preferably contain between 1 and 5 g. per liter of the alkylalkoxy alkyl cellulose. Furthermore, pH value of the liquor should preferably be adjusted to be between 3 and 5 and the liquor may also contain normal condensation catalysts such as magnesium chloride, aluminum chloride, ammonium chloride, ammonium nitrate, borax, etc.

Among the suitable resin-forming substances for the purpose of the present invention are formaldehyde or glyoxal (the glyoxal preferably being used together with an aldehyde carboxylic acid such as glyoxylic acid as condensation catalyst), urea-formaldehyde pre-condensates such as methylol urea, dimethylol urea, melamine-formaldehyde condensates, methylol biuret, dimethylol biuret, the reaction product in neutral to slightly alkaline medium of methylol urea and glyoxal and similar products.

The textile material which has been treated with the liquor in accordance with the present invention, which actually have been impregnated with the liquor, for example by spraying the liquor onto the textile material or preferably by immersing the material in the liquor, is treated to remove the excess of liquor for example by pressing or by centrifuging the material and this predried textile material can be heated to a temperature up to 150° C. depending upon the duration of heating. The drying and heating can also be carried out in a single step.

The following examples are given to illustrate the present invention. The scope of the invention is not, however, meant to be limited to the specific details of the examples.

#### EXAMPLE I

Copy fabric is immersed in a liquor which in each liter contains 150 g. of the reaction product of methylol urea and glyoxal in neutral to weakly alkaline medium, 10 g. of magnesium chloride as catalyst and 2 g. of ethyloxyethyl cellulose (the mol ratio of the components used to form the cellulose, calculated on the glucose anhydride, of cellulose to ethyl chloride to ethylene oxide with 1:1:3). The bath temperature is 35-40° C., the pH value of the treatment solution is 3.5. The steeped material is pressed, dried and heated to a temperature of 145° C. for 7 minutes.

For comparison purposes, samples of the same cotton fabric were treated under the same conditions with liquors which instead of containing the etherified cellulose ethyloxyethyl cellulose in a mol ratio of 1:1:3, contained ethyloxy cellulose which was produced in a ratio of cellulose (calculated as glucose anhydride) to ethyl chloride to ethylene oxide in a mol ratio of 1:1:2 and in another test in a mol ratio of 1:1:4.

The crease angles in weft and warp threads and the feel characteristics of the treated samples and of the untreated samples were determined and are set forth in the following table:

Table 1

| Cellulose mixed ether, mol ratio of cellulose:ethyl chloride:alkylene oxide | Crease angle in degrees—dry |                                      | Crease angle in degrees—wet |                                      | Feel       |
|-----------------------------------------------------------------------------|-----------------------------|--------------------------------------|-----------------------------|--------------------------------------|------------|
|                                                                             | Before laundering           | After 5 launderings in boiling water | Before laundering           | After 5 launderings in boiling water |            |
| 1:1:3.....                                                                  | 129/124                     | 118/121                              | 143/131                     | 124/114                              | Very good. |
| 1:1:2.....                                                                  | 86/86                       | 80/79                                | 129/120                     | 110/105                              | Limp.      |
| 1:1:4.....                                                                  | 116/107                     | 95/99                                | 144/146                     | 115/116                              | Do.        |
| Untreated material.....                                                     | 101/108                     | 91/99                                | 124/121                     | 110/108                              | Do.        |

The treatment of cellulose poplin with the above set forth liquors under the same conditions gave the results set forth in Table 2.

Table 2

| Cellulose mixed ether, mol ratio of cellulose:ethyl chloride:alkylene oxide | Crease angle in degrees—dry |                                      | Crease angle in degrees—wet |                                      | Feel          |
|-----------------------------------------------------------------------------|-----------------------------|--------------------------------------|-----------------------------|--------------------------------------|---------------|
|                                                                             | Before laundering           | after 5 launderings in boiling water | Before laundering           | After 5 launderings in boiling water |               |
| 1:1:3.....                                                                  | 115/116                     | 113/116                              | 124/127                     | 135/137                              | Very good.    |
| 1:1:2.....                                                                  | 104/102                     | 109/101                              | 109/101                     | 140/145                              | Insufficient. |
| 1:1:4.....                                                                  | 104/107                     | 110/107                              | 93/100                      | 115/110                              | Do.           |
| Untreated material.....                                                     | 109/107                     | 100/106                              | 116/130                     | 125/120                              | Limp.         |

Further comparative tests were carried out using liquors (a) without cellulose derivative, (b) with 2 g. per liter of carboxy methyl cellulose instead of the cellulose mixed ether, (c) with the 2 g. per liter of the cellulose mixed ether, that is the ethyloxyethyl cellulose of the mol ratio 1:1:3, and a cellulose poplin was treated with the different liquors. The results were compared and also compared with (d) untreated material, these results being set forth in Table 3 below.

Table 3

| Liquor                                               | Crease before laundering |                    | Angle in degrees after boiling wash | Shearing strength, turns | Feel |
|------------------------------------------------------|--------------------------|--------------------|-------------------------------------|--------------------------|------|
|                                                      | Before laundering        | after boiling wash |                                     |                          |      |
| Without cellulose derivative.....                    | 140/141                  | 124/126            | 580                                 | Limp.                    |      |
| 2 g./l. carboxymethylcellulose.....                  | 128/130                  | 118/107            | 623                                 | Do.                      |      |
| 2 g./l. cellulose mixed ether, mol ratio, 1:1:3..... | 148/150                  | 139/134            | 780                                 | Very good.               |      |
| Untreated material.....                              | 84/88                    | .....              | 1,057                               | Limp.                    |      |

For the production of the cellulose mixed ether with the mol ratio of cellulose to ethylchloride to ethylene oxide of 1:1:3 (calculating the cellulose as glucose anhydride), pine sulfite cellulose at a temperature of 18 to 20° C. is immersed for 1 hour in 19% sodium hydroxide, pressed under a pressing factor of 30 and comminuted for an hour. 75 g. of the obtained, unripened alkali cellulose are shaken in a shaken autoclave of 2 liter capacity with 9.96 g. of fluid ethylchloride, 20.3 g. of liquefied ethylene oxide and 1 liter of peroxide-free tetrahydrofuran at a temperature of 80° C. for 5 hours.

The yellowish brown reaction product is filtered off by suction, pressed sharply and dried under vacuum over calcium chloride. The product is easily soluble in cold water and no fiber residue remains upon dissolution. The yield of the dry reaction product is 60 to 65 g. The diluting agent must be peroxide-free. To remove the peroxide the tetrahydrofuran is allowed to stand with concentrated potassium hydroxide with shaking from time to time, and after separation of the potassium hydroxide liquor is rectified.

#### EXAMPLE II

A treating liquid is used containing per liter 100 grams of technical glyoxal (consisting of 20% glyoxalic acid, 50% acetic acid and 30% glyoxal), 25 grams of technical borax and 2 grams of an ethyloxyethyl cellulose (molar relationship 1:1:3) prepared as described in Example I. The solution has a pH of 3.7.

A rayon shirt material having a crease angle of 76° in the warp and of 81° in the weft and a rub resistance of 1075 passes (at 500 grams preload) is treated in the above treating liquid for two minutes, thereafter pressed to 90% moisture content and then dried at 90° C.

The thus treated goods were found to have in warp and weft, respectively, a crease angle of 157°/151°, after one washing with sodium lauryl sulfonate of 119°/121°, and a rub resistance value of 779.

A sample of the same material was treated under the same conditions as described above, with a treating liquid of the above described composition, however omitting the mixed cellulose ether. The dried material showed the following values:

Crease angle 145°/147°, or 110°/110° after one washing with sodium lauryl sulfonate; rub resistance: 664 passes (with 500 grams preload).

### EXAMPLE III

A rayon shirt material as described in Example II is soaked in a treating liquid containing 90 grams of the reaction product obtained by reaction of dimethylol urea and glyoxal in aqueous solution at a pH of 7.5, 11.5 grams of  $\text{AlCl}_3 \cdot 6\text{H}_2\text{O}$ , 10 grams of boric acid and 2 grams of the mixed cellulose ether described in Example II. The pH of the treating liquid is 3.6. Liquid is squeezed off to a residual moisture content of 100% and the material is then dried at between 100 and 110° C.

The thus treated material has a crease angle of 123°/115°, or of 108°/120° after one washing with sodium lauryl sulfonate, a rub resistance of 890 and pleasant soft feel (touch).

A sample of the same material was finished under identical conditions with the exception that the treating liquid did not contain a mixed cellulose ether. The dried goods had the following dry-crease angle:

103°/108°, or 93°/91° after one washing with sodium lauryl sulfonate; rub resistance was 856 passes with 500 gram preload.

### EXAMPLE IV

An aqueous 33.5% formaldehyde solution is adjusted with sodium carbonate to a pH of between 8.5 and 9.0. 173 grams of this solution are then mixed with 105 grams biuret. The mixture is heated to between 50 and 60° C. until the biuret is completely dissolved. 170 grams of the thus obtained solution are mixed with 830 grams water, and 2 grams of the mixed cellulose ether of Example III are added thereto. This treating liquid is then adjusted with concentrated hydrochloric acid to a pH of 5.7 under the addition of 8 grams  $\text{NH}_4\text{NO}_3$ .

A sample of the rayon shirt material of Example III is then soaked at a temperature of about 35° in this solution which has a pH of 5.7. The material is then squeezed and dried at 100° C. and thereafter hardened for six minutes at 130° C.

The crease angles in warp and weft of the thus finished material are 144°/133°, or 114°/119° after one washing with sodium lauryl sulfonate; rub resistance: 670.

The material finished with the same treating liquid except for the absence of cellulose ether and under otherwise similar conditions has a crease angle of 128°/131°, or 111°/111° after one washing with sodium lauryl sulfonate, and a rub resistance of 659.

### EXAMPLE V

A treating liquid is prepared which contains per liter 100 grams of dimethylol urea 100%, 5 grams of  $\text{NH}_4\text{NO}_3$  and 2 grams of the ethyloxyethyl cellulose (molar relationship 1:1:3) similar to the ether used in Example III. A sample of the rayon shirt material of Example III is soaked in this treating liquid and after removal of excess liquid by squeezing, the sample is subjected to a single drying step carried out for five minutes at 130° C.

The crease angles in warp and weft of the treated material are 142°/140°, or 122°/130° after one washing with sodium lauryl sulfonate. Rub resistance: 610. A sample of similar material finished with a treating liquid free of the addition of cellulose ether has crease angles of 129°/129°, or 115°/127° after one washing with sodium lauryl sulfonate. Rub resistance: 540.

Without further analysis, the foregoing will so fully reveal the gist of the present invention that others can by applying current knowledge readily adapt it for various applications without omitting features that, from the

standpoint of prior art, fairly constitute essential characteristics of the generic or specific aspects of this invention and, therefore, such adaptations should and are intended to be comprehended within the meaning and range of equivalence of the following claims.

What is claimed as new and desired to be secured by Letters Patent is:

1. Method of improving properties such as the crease resistance and non-shrinking properties of cellulose textiles, comprising the steps of treating a cellulose textile material with an acid aqueous liquor containing in solution a water soluble resin-forming substance which upon heating to a predetermined temperature below the temperature at which damage to said cellulose textile material occurs is transformed into an insoluble resinous substance, said water soluble resin-forming substance containing hydroxyl groups, and also containing in solution a water soluble alkyloxy alkyl cellulose mixed ether containing ether groups and also containing free hydroxyl groups formed by the reaction of an alkali cellulose with about 1 mol of an alkylating agent and about 3 mols of an alkoxylating agent calculated per each mol of glucose anhydride of said alkali cellulose; and heating the thus treated cellulose textile material to said predetermined temperature so as to convert said water soluble resin-forming substance into an insoluble resinous substance and to cause cross linking reaction between the same and said water soluble alkyloxy alkyl cellulose, thereby forming a treated cellulose textile material having improved properties.
2. Method of improving properties such as the crease resistance and non-shrinking properties of cellulose textiles, comprising the steps of treating a cellulose textile material with an acid aqueous liquor containing in solution a water soluble resin-forming substance which upon heating to a temperature between 100 and 150° C. is transformed into an insoluble resinous substance, said water soluble resin-forming substance containing hydroxyl groups, and also containing in solution a water soluble alkyloxy alkyl cellulose mixed ether containing ether groups and also containing free hydroxyl groups formed by the reaction of an alkali cellulose with about 1 mol of an alkylating agent and about 3 mols of an alkoxylating agent calculated per each mol of glucose anhydride of said alkali cellulose; and heating the thus treated cellulose textile material to said temperature so as to convert said water soluble resin-forming substance into an insoluble resinous substance and to cause cross linking reaction between the same and said water soluble alkyloxy alkyl cellulose, thereby forming a treated cellulose textile material having improved properties.
3. Method of improving properties such as the crease resistance and non-shrinking properties of cellulose textiles, comprising the steps of treating a cellulose textile material with an acid aqueous liquor containing in solution a water soluble resin-forming substance which upon heating to a predetermined temperature below the temperature at which damage to said cellulose textile material occurs is transformed into an insoluble resinous substance, said water soluble resin-forming substance containing hydroxyl groups, and also containing in solution a water soluble alkyloxy alkyl cellulose mixed ether containing ether groups and also containing free hydroxyl groups formed by the reaction of an alkali cellulose with about 1 mol of a lower alkyl halogenide as an alkylating agent and about 3 mols of a lower alkylene oxide as an alkoxylating agent calculated per each mol of glucose anhydride of said alkali cellulose; and heating the thus treated cellulose textile material to said predetermined temperature so as to convert said water soluble resin-forming substance into an insoluble resinous substance and to cause cross linking reaction between the same and said water soluble alkyloxy alkyl cellulose, thereby forming a treated cellulose textile material having improved properties.

4. Method of improving properties such as the crease resistance and non-shrinking properties of cellulose textiles, comprising the steps of treating a cellulose textile material with an acid aqueous liquor containing in solution a water soluble resin-forming substance which upon heating to a predetermined temperature below the temperature at which damage to said cellulose textile material occurs is transformed into an insoluble resinous substance, said water soluble resin-forming substance containing hydroxyl groups, and also containing in solution a water soluble alkyloxy alkyl cellulose mixed ether containing ether groups and also containing free hydroxyl groups formed by the reaction of an alkali cellulose with about 1 mol of an alkylating agent selected from the group consisting of methyl bromide, methyl chloride, ethyl bromide and ethyl chloride and about 3 mols of an alkoxylating agent selected from the group consisting of ethylene oxide, propylene oxide and ethylene chlorohydrin calculated per each mol of glucose anhydride of said alkali cellulose, and heating the thus treated cellulose textile material to said predetermined temperature so as to convert said water soluble resin-forming substance into an insoluble resinous substance and to cause cross linking reaction between the same and said water soluble alkyloxy alkyl cellulose, thereby forming a treated cellulose textile material having improved properties.

5. Method of improving properties such as the crease resistance and non-shrinking properties of cellulose textiles, comprising the steps of treating a cellulose textile material with an acid aqueous liquor containing in solution a water soluble resin-forming substance which upon heating to a predetermined temperature below the temperature at which damage to said cellulose textile material occurs is transformed into an insoluble resinous substance, said water soluble resin-forming substance containing hydroxyl groups, and also containing in solution 1-5 g. per liter of a water soluble alkyloxy alkyl cellulose mixed ether containing ether groups and also containing free hydroxyl groups formed by the reaction of an alkali cellulose with about 1 mol of an alkylating agent and about 3 mols of an alkoxyating agent calculated per each mol of glucose anhydride of said alkali cellulose; and heating the thus treated cellulose textile material to said predetermined temperature so as to convert said water soluble resin-forming substance into an insoluble resinous substance and to cause cross linking reaction between the same and said water soluble alkyloxy alkyl cellulose, thereby forming a treated cellulose textile material having improved properties.

6. Method of improving properties such as the crease resistance and non-shrinking properties of cellulose textiles, comprising the steps of treating a cellulose textile material with an acid aqueous liquor containing in solution a water soluble resin-forming substance which upon heating to a temperature between 100 and 150° C. is transformed into an insoluble resinous substance, said water soluble resin-forming substance containing hydroxyl groups, and also containing in solution 1-5 g. per liter of a water soluble alkyloxy alkyl cellulose mixed ether containing ether groups and also containing free hydroxyl groups formed by the reaction of an alkali cellulose with about 1 mol of an alkylating agent selected from the group consisting of methyl bromide, methyl chloride, ethyl bromide and ethyl chloride and about 3 mols of an alkoxylating agent selected from the group consisting of ethylene oxide, propylene oxide and ethylene chlorohydrin calculated per each mol of glucose anhydride of said alkali cellulose; and heating the thus treated cellulose textile material to said temperature so as to convert said water soluble resin-forming substance into an insoluble resinous substance and to cause cross linking reaction between the same and said water soluble alkyloxy alkyl cellulose, thereby forming a treated cellulose textile material having improved properties.

7. Method of improving properties such as the crease  
resistance and non-shrinking properties of cellulose tex-  
tiles, comprising the steps of treating a cellulose textile  
material with an acid aqueous liquor having a pH be-  
5 between 3 and 5 and containing in solution a water soluble  
resin-forming substance which upon heating to a tempera-  
ture between 100 and 150° C. is transformed into an  
insoluble resinous substance, said water soluble resin-  
forming substance containing hydroxyl groups, and also  
10 containing in solution a water soluble alkyloxy alkyl cel-  
lulose mixed ether containing ether groups and also con-  
taining free hydroxyl groups formed by the reaction of  
an alkali cellulose with about 1 mol of an alkylating agent  
and about 3 mols of an alkoxylating agent calculated per  
15 each mol of glucose anhydride of said alkali cellulose;  
and heating the thus treated cellulose textile material to  
said temperature so as to convert said water soluble  
resin-forming substance into an insoluble resinous sub-  
stance and to cause cross linking reaction between the  
20 same and said water soluble alkyloxy alkyl cellulose,  
thereby forming a treated cellulose textile material hav-  
ing improved properties.

8. Method of improving properties such as the crease  
resistance and non-shrinking of cellulose textiles, com-  
25 prising the steps of treating a cellulose textile material  
with an acid aqueous liquor having a pH between 3 and  
5 and containing in solution a water soluble resin-form-  
ing substance which upon heating to a predetermined  
temperature below the temperature at which damage to  
30 said cellulose textile material occurs is transformed into  
an insoluble resinous substance, said water soluble resin-  
forming substance containing hydroxyl groups, and also  
containing in solution a water soluble alkyloxy alkyl cel-  
lulose mixed ether containing ether groups and also con-  
35 taining free hydroxyl groups formed by the reaction of  
an alkali cellulose with about 1 mol of an alkylating  
agent selected from the group consisting of methyl bro-  
mide, methyl chloride, ethyl bromide and ethyl chloride  
and about 3 mols of an alkoxylating agent selected from  
40 the group consisting of ethylene oxide, propylene oxide  
and ethylene chlorohydrin calculated per each mol of  
glucose anhydride of said alkali cellulose; and heating  
the thus treated cellulose textile material to said pre-  
determined temperature so as to convert said water soluble  
45 resin-forming substance into an insoluble resinous sub-  
stance and to cause cross linking reaction between the  
same and said water soluble alkyloxy alkyl cellulose,  
thereby forming a treated cellulose textile material hav-  
ing improved properties.

50 9. Method of improving properties such as the crease resistance and non-shrinking properties of cellulose textiles, comprising the steps of treating a cellulose textile material with an acid aqueous liquor having a pH between 3 and 5 and containing in solution a water soluble resin-forming substance which upon heating to a temperature between 100 and 150° C. is transformed into an insoluble resinous substance, said water soluble resin-forming substance containing hydroxyl groups, and also containing in solution 1-5 g. per liter of a water soluble 55 alkyloxy alkyl cellulose mixed ether containing ether groups and also containing free hydroxyl groups formed by the reaction of an alkali cellulose with about 1 mol of an alkylating agent selected from the group consisting of methyl bromide, methyl chloride, ethyl bromide and ethyl chloride and about 3 mols of an alkyoxylating agent selected from the group consisting of ethylene oxide, propylene oxide and ethylene chlorohydrin calculated per each mol of glucose anhydride of said alkali cellulose; and heating the thus treated cellulose textile material to said temperature so as to convert said water soluble resin-forming substance into an insoluble resinous substance and to cause cross linking reaction between the same and said water soluble alkyloxy alkyl cellulose, thereby forming a treated cellulose textile material having improved properties.

10. Method of improving properties such as the crease resistance and non-shrinking properties of cellulose textiles, comprising the steps of treating a cellulose textile material with an acid aqueous liquor containing in solution a water soluble resin-forming substance selected from the group consisting of formaldehyde, glyoxal, dimethylol urea, methylol urea, melamine-formaldehyde condensate, methylol biuret, dimethylol biuret and the reaction product of methylol urea and glyoxal which upon heating to a predetermined temperature below the temperature at which damage to said cellulose textile material occurs is transformed into an insoluble resinous substance, said water-soluble resin-forming substance containing hydroxyl groups, and also containing in solution a water soluble alkyloxy alkyl cellulose mixed ether containing ether groups and also containing free hydroxyl groups formed by the reaction of an alkali cellulose with about 1 mol of an alkylating agent and about 3 mols of an alkoxylation agent calculated per each mol of glucose anhydride of said alkali cellulose; and heating the thus treated cellulose textile material to said predetermined temperature so as to convert said water soluble resin-forming substance into an insoluble resinous substance and to cause cross linking reaction between the same and said water soluble alkyloxy alkyl cellulose, thereby forming a treated cellulose textile material having improved properties.

11. Method of improving properties such as the crease resistance and non-shrinking properties of cellulose textiles, comprising the steps of treating a cellulose textile material with an acid aqueous liquor having a pH be-

tween 3 and 5 and containing in solution a water soluble resin-forming substance selected from the group consisting of formaldehyde, glyoxal, dimethylol urea, methylol urea, melamine-formaldehyde condensate, methylol biuret, dimethylol biuret and the reaction product of methylol urea and glyoxal which upon heating to a temperature between 100 and 150° C. is transformed into an insoluble resinous substance, said water soluble resin-forming substance containing hydroxyl groups, and also containing in solution a water soluble alkyloxy alkyl cellulose containing ether groups and also containing free hydroxyl groups formed by the reaction of an alkali alkyl cellulose mixed ether with about 1 mol of an alkylating agent and about 3 mols of an alkoxylation agent calculated per each mol of glucose anhydride of said alkali cellulose; and heating the thus treated cellulose textile material to said temperature so as to convert said water soluble resin-forming substance into an insoluble resinous substance and to cause cross linking reaction between the same and said water soluble alkyloxy alkyl cellulose, thereby forming a treated cellulose textile material having improved properties.

## References Cited in the file of this patent

## UNITED STATES PATENTS

|           |                |               |
|-----------|----------------|---------------|
| 1,505,043 | Lilienfeld     | Aug. 12, 1924 |
| 2,190,451 | Haskins        | Feb. 13, 1940 |
| 2,469,431 | Broderick      | May 10, 1949  |
| 2,644,818 | Downing et al. | July 7, 1953  |
| 2,672,427 | Bauling et al. | Mar. 16, 1954 |
| 2,949,452 | Savage         | Aug. 16, 1960 |